

## UNITED STATES PATENT OFFICE

2,614,024

## THIOFORMALDEHYDE AND MERCURIC CHLORIDE TREATMENT OF PROTEIN FILAMENTS

George K. Simpson, Fairlie, and David Traill, Ardrossan, Scotland, assignors to Imperial Chemical Industries Limited, a corporation of Great Britain

No Drawing. Application February 4, 1949, Serial No. 74,724. In Great Britain March 3, 1948

7 Claims. (Cl. 8—127.6)

1

The present invention is concerned with the provision of a method for improving the strength of artificial protein filaments treated with reagents capable of forming in situ nascent monomeric thioformaldehyde as for example, according to United States Patent No. 2,319,009 so as to permit them to be readily processed in the existing machinery employed in the manufacture of textile products.

United States Patent No. 2,319,009 describes and claims inter alia the treatment of coagulated casein or vegetable seed protein filaments with a concentrated aqueous solution of a salt of a hydrohalide containing formaldehyde, or a compound which will yield formaldehyde under the conditions of the treatment, a salt of a reducing sulphur acid in which the atomic proportion, reckoned on the anhydrous salt, of oxygen if present, to sulphur does not exceed 2:1, and an acid which does not oxidize the salt of the sulphur acid, and which is substantially completely ionized in dilute aqueous solution.

While it is known that stretching of coagulated wet spun filaments previous to their insolubilization, for example by means of formaldehyde in the presence of an acidified highly concentrated aqueous saline solution, has a beneficial effect on the strength of the insolubilized filaments produced, and that the strength of the insolubilized filaments, can frequently be further increased by treatments involving further stretching, such stretching processes as have heretofore been disclosed with respect to protein fibers not only do not permit the application of extensive stretching but the effects produced are only relatively small.

In our copending application Serial No. 45,794, filed August 23, 1948, now Patent 2,535,103, we have described a method for improving the strength of artificial protein filaments which have been insolubilized by treatment with formaldehyde by treating these insolubilized filaments while under tension in an aqueous solution of an ionizable mercuric salt.

We have now found that filaments of very marked improved strength are obtained if coagulated protein filaments treated according to United States Patent No. 2,319,009, if desired washed to free them from surface and uncombined acid or formaldehyde, are treated under tension with an aqueous solution containing mercuric chloride.

According to the present invention, therefore, the method of improving the strength of artificial protein filaments treated with reagents

2

capable of forming in situ nascent monomeric thioformaldehyde as for example according to United States Patent No. 2,319,009 comprises treating the said protein filaments under tension with an aqueous solution of mercuric chloride.

The aqueous solution of mercuric chloride is preferably at a temperature between 70° C. and 80° C. and is preferably acidified with hydrochloric acid.

10 The protein filaments treated according to United States Patent No. 2,319,009 are preferably stretched to about 350 per cent while undergoing treatment in an aqueous solution of mercuric chloride.

15 The treatment according to the invention can reduce the diameter of the filaments by about 9 $\mu$  and can increase the wet strength of the filament by about 60 per cent.

20 Protein filaments treated according to United States Patent No. 2,319,009 tend to have low elongation at break in the dry state and high elongation when wet. Treatment according to the present invention improves these properties, that is to say the fibres become less brittle when dry and less plastic when wet.

25 The invention is illustrated by the following example.

30 A solution of ground nut protein in caustic soda is extruded into a sulphuric acid/sodium sulphate coagulating bath. These fibres are now given an insolubilizing treatment for 16 hours at 38° C. in a solution consisting of 960 ml. brine, 30 ml. formalin, 40 ml. conc. hydrochloric acid and 32.5 gm. sodium sulphide ( $\text{Na}_2\text{S} \cdot 9\text{H}_2\text{O}$ ). The fibres are now washed free from acid and dried at 110° C. The insolubilized tow thus obtained is now stretched to a maximum in a bath containing 3% mercuric chloride and 0.1 N hydrochloric acid at 70° C. The stretch is maintained for about 30 minutes and the tow is then washed in running water and dried at 108° C.

35 The sulphide-insolubilized filaments treated with mercuric chloride in this manner are increased in wet strength to about 60 per cent and the increase of elongation at break when dry is about 200 per cent. The elongation at break when wet is decreased by 50 per cent.

40 It will be appreciated that the term "insolubilized," as used in the appended claims, is intended to mean filaments which have been treated with thioformaldehyde so as to be substantially unaffected when exposed to the resistance test outlined on page 2, column 2, lines 55 through 61, of U. S. Patent No. 2,319,009, i. e., the 45 filaments should be substantially unaffected by

treatment for 90 minutes at 97° C. with a bath containing 0.1% sulfuric acid and 0.25% sodium sulfate. The filaments being treated are, therefore, to be distinguished from hardened portein filaments, i. e., filaments which are insoluble in cold water but are affected adversely in boiling water and hot dilute acid. In other words, the insolubilized protein filaments with which the present application is concerned are not only insoluble in cold water, but are also resistant to 10 boiling water and hot dilute acid.

We claim:

1. A method of improving the strength of artificial protein filaments selected from the group consisting of casein and vegetable seed protein 15 filaments which have been insolubilized by treatment with nascent monomeric thioformaldehyde formed in situ which comprises stretching said insolubilized protein filaments while in an aqueous solution of mercuric chloride under 20 conditions sufficient to effect a substantial increase in the wet strength and dry elongation at break of said filaments.

2. The method of claim 1, wherein the aqueous solution of mercuric chloride is at a temperature of between 70° and 80° C. 25

3. The method of claim 1, wherein the aqueous solution of mercuric chloride is acidified with hydrochloric acid.

4. The method of claim 1, wherein the insolubilized protein filaments are stretched to about 350% of their original length, while in the aqueous solution of mercuric chloride.

5. A method of improving the strength of artificial protein filaments selected from the group consisting of casein and vegetable seed protein 35 filaments which have been insolubilized by treatment with nascent monomeric thioformaldehyde formed in situ which comprises stretching said insolubilized protein filaments to about 40 350% of their original length in an aqueous solution of mercuric chloride and hydrochloric acid

at a temperature of between 70° and 80° C., using a concentration of chloride and a time of treatment sufficient to effect a substantial increase in wet strength and dry elongation at break of said filaments.

6. The method of claim 5, wherein said protein filaments are ground nut protein filaments.

7. The artificial protein filaments of improved strength obtained by the method described in claim 1, said filaments being characterized by having an increased wet strength and increased elongation at break when dry.

GEORGE K. SIMPSON.  
DAVID TRAILL.

#### REFERENCES CITED

The following references are of record in the file of this patent:

#### UNITED STATES PATENTS

| Number    | Name              | Date          |
|-----------|-------------------|---------------|
| 339,348   | Tweedy            | Apr. 6, 1886  |
| 998,341   | Illingsworth      | July 18, 1911 |
| 1,799,047 | Jones             | Mar. 31, 1931 |
| 2,297,397 | Feretti           | Mar. 2, 1940  |
| 2,319,009 | McLean            | May 11, 1943  |
| 2,374,201 | Highberger et al. | Apr. 24, 1945 |

#### FOREIGN PATENTS

| Number  | Country       | Date          |
|---------|---------------|---------------|
| 508,781 | Great Britain | June 26, 1939 |

#### OTHER REFERENCES

Synthetic Tannins, G. Grasser and Enna, Cross by Lockwood and Son, London (1922), page 75.

"A Study on Chronic Mercurialism in the Hatters' Fur-Cutting Industry," page 38 of Public Health Bulletin Number 234, U. S. Public Health Service.

"News Edition—Amer. Chem. Soc.," November 25, 1941, article by Beal et al. Pages 1239 and 1242. 8-112.